

1

2,913,788

## METHOD OF CASTING INGOTS

Robert E. Kramig, Jr., Cincinnati, Ohio; Anna Louise Kramig, executrix and trustee of the estate of said Robert E. Kramig, Jr., deceased

No Drawing. Application May 18, 1953  
Serial No. 355,880

3 Claims. (Cl. 22—200)

This invention relates to the casting of ingots of steel, iron and other metals. The invention is addressed particularly to the problem of preventing the adherence of an ingot casting to the stool upon which the ingot mold is mounted, and to prevent deterioration of the stool by the molten metal during casting.

In the fabrication of sheets and shapes of steel, it is conventional procedure to first produce an ingot from the molten and refined metal. For this purpose, a tubular tapered ingot mold is placed vertically upon a large heavy plate or so-called stool which is made of cast iron, the upper surface of the plate forming the bottom closure of the mold cavity. Molten metal at a temperature of approximately 3400° F. is poured into the cavity from a ladle and is allowed to cool and solidify within the cavity. Subsequently, the ingot mold and the contained casting is lifted from the plate and removed to another place where the mold is separated from the casting. An empty ingot mold is later placed upon the plate for the production of another ingot. The ingots produced in this manner vary, depending upon mold size, from approximately 5 to 10 tons, and the stool is proportionately large and massive.

In steel manufacture by this procedure, it is apparent that the surface of the stool is exposed directly to the very high temperature of the stream of molten steel which is poured against it. One function of the stool, aside from providing a support for the ingot mold, is to conduct heat from the metal of the casting so that it may cool at a suitably rapid rate. However, at the beginning of a pouring operation, the hot metal which comes into direct engagement with the surface of the stool, at the velocity which it attains in falling from a height of seven feet or more, causes the surface metal of the stool to become melted and dislodged. For this reason, a crater is produced in the stool surface, the size of the crater becoming progressively larger following each pouring operation. For this reason, it is requisite that the stools be replaced from time to time, which, in view of their substantial size, involves considerable expense.

Under ideal conditions, the relatively low temperature of the stool at the start of a pouring operation is sufficient to prevent actual adhesion of the cast ingot to the stool surface. However, it frequently occurs that the molten metal actually integrates itself with the metal of the stool, as though the two became welded together. In this event, it is impossible to lift the ingot from the stool and it then becomes necessary to separate the stool from the ingot by whatever means may be required; usually, the entire assembly is removed to a yard where the stool can be pounded upon with a heavy weight in order to break the weldments where the ingot and stool are seized together. Such operations are obviously costly and interfere with orderly production.

In order to facilitate the parting of the ingot casting from the stool after solidification of the casting, it has been conventional procedure in some steel plants to

2

throw a layer of calcium carbide over the stool surface. To some extent, this procedure reduces the frequency with which so-called "stickers" occur. However, the heavy stream of molten metal which falls against the stool surface flushes away the light powder layer with the result that this expedient, though helpful, has by no means either cured the problem of preventing adherence of the casting to the stool or the problem of preventing cratering of the stool surface by the molten metal.

Other expedients have also been proposed, such as recessing the stool surface at the area thereof which normally receives the falling stream of metal and of placing a block of carbon in the recess so as to enable carbon to insulate the metal of the stool against the deteriorating effects of the molten metal stream. In this practice, however, it is found that the molten steel dissolves or absorbs carbon from the target block and, therefore, the steel first poured into the mold is different metallurgically from the metal in the balance of the ingot.

It has also been proposed to use a wound coil of strap steel as the target at the bottom of the mold against which the falling stream can be directed. In this arrangement, it is intended that the steel of the target be melted by the molten steel of the casting and thereby absorbed within it, meanwhile chilling the adjacent molten steel sufficiently to prevent seizure or sticking. However, targets of this type introduce metallurgical variations into the steel ingot and are not reliable in the performance of their intended function.

Various heat insulating compositions which might be sufficiently refractory to withstand the high temperature at which the steel is poured are undesirable because they interfere with the intended conductance of heat from the casting to the steel.

This invention is based upon the paradoxical determination that a resin-laminated asbestos plate placed over the stool face at the bottom of an ingot mold is capable of protecting the stool face against cratering by the molten metal, is capable of preventing so-called "stickers" or adhesion of the metal of the ingot casting to the stool, and is also capable of providing the desired conductance of heat from the casting to the stool plate so that cooling of the casting at a normal rate may be achieved.

The practice of this invention, therefore, contemplates the disposition of a densely compacted layer of bonded asbestos fibers within the mold, either over the entire bottom area thereof or at that area thereof against which the stream of molten metal is directed at the start of the pouring operation. The bonding agent, if resinous, as is preferred, carbonizes under the intense heat to which it is subjected, but the carbon with which the molten steel comes into contact in this manner does not change the metallurgical composition of the steel in appreciable degree, either because the carbon is not adequate in amount or because it is retained by the asbestos fibers to such a degree that substantial dissolution thereof within the steel does not occur.

A plate of this type may be called a "smirch plate," suffering destruction as an incident to the pouring of the molten metal into the mold cavity but coincidentally protecting the stool against cratering and adhesion of the casting thereto while also providing the desired heat conductance to the stool. The cost of such a plate is low in comparison with the costs that are involved in stool replacement or in separating a seized casting from a stool, and is also low in comparison with the cost of the various expedients which heretofore have been proposed but found to be only partially effective.

Asbestos is nominally considered a good heat insulator; this is confirmed by its extensive usage on boilers,

pipes and elsewhere where heat transmission is to be prevented. Actually, however, it is found that densely compacted asbestos fibers bonded into intimate contact by a synthetic resin has high heat conductance properties. The asbestos fibers themselves are of refractory nature, but the resin in the bond is rapidly decomposed into elemental carbon at temperatures of the type in question. Even though this decomposition of the bond occurs within the mold, the residual asbestos fibers still provide the conductance of heat from the casting to the stool metal, with the result that the desired rate of cooling is attained.

An important characteristic of the smirch plates of the present invention is that they are capable of retaining their physical integrity throughout the initial period when first subjected to the impact of the falling stream of molten steel. As soon as steel is poured into the mold to a depth of two or three inches, this liquid layer protects the smirch plate against the attrition of the falling stream, and what happens thereafter to the smirch plate is of no consequence.

A typical smirch plate of the present invention is fabricated conveniently from asbestos paper which is coated with synthetic resin of, for example, the phenol formaldehyde type, then laminated with similar layers until an assembly of suitable thickness is built up, after which the assembly is placed in a press where it is cured under a pressure of several hundred pounds per square inch or more, to thermally set the resin. During curing, the pressure which is exerted upon the laminate assembly causes migration of the resin and coincident compaction of the asbestos fibers one to another, and the resin also becomes thermally set.

A smirch plate produced in this manner may be from  $\frac{1}{8}$  of an inch in thickness to  $\frac{1}{4}$  of an inch or more, depending upon the relative size of the ingot mold with which it is to be used.

Various synthetic resins may be used as the bonding medium for the asbestos fibers of the smirch plate, the phenol formaldehyde resins generally being the cheapest to use and, therefore, preferred. Resin content may constitute from approximately 15% to 30% by weight of the finished plate. If the resin content is much below 15%, the bonding of the fibers is not usually sufficient to provide the physical integrity which is requisite to enable the plate to withstand destruction during the initial pouring of the ingot, whereas a resin content above approximately 30% merely increases cost without providing commensurate advantage, and, in fact, is undesirable to the extent that the excess merely introduces an additional quantity of carbon at the end of the ingot, which might be undesirable metallurgically.

Phenol formaldehyde resin conveniently may be employed in the form of an aqueous dispersion of approximately 80% resin content applied either by coating or immersion or in other suitable manner to the asbestos. Resin in particle or granular form or in other than aqueous medium also may be used. It is to be noted, however, that whatever vehicle is employed for the purpose of distributing the resin upon the asbestos be removed before use of the final product, either by predrying before curing or by vapor liberation during curing. The presence of moisture or solvents in the finished product will, of course, cause violent vapor liberation of the smirch plate during use with resultant rupture of the plant laminations or fibers.

Commercial grades of asbestos paper constitute a convenient source of asbestos fibers; a six pound commercial asbestos paper, for example, has been found to be satisfactory. To make a smirch plate approximately  $\frac{1}{4}$  of an inch in thickness, approximately twenty layers of asbestos paper, each coated with synthetic resin may be used, with curing under a pressure of approximately 250 pounds per square inch, at a temperature of about 325° F. for a period of twenty to thirty minutes or more. Unit pressure which is maintained upon the plate during

the curing of the resin will, of course, govern the degree of compaction of the fibers, the greater the pressure the more dense and the less thick the resulting sheet will be.

Under a curing pressure of approximately 250 pounds per square inch, with a resin content of 20%, a smirch plate approximately  $\frac{1}{4}$  of an inch thick is produced which displays remarkable heat resistance. Such a plate, for example, is capable of surviving direct heat of an oxy-acetylene torch for a period of sixty-five seconds before penetration of the torch flame through the sheet. A similar plate only  $\frac{1}{8}$  of an inch thick resists penetration by the flame for a period of approximately twenty seconds. Inasmuch as the pouring of molten metal into an ingot mold is usually completed in a period of from approximately thirty to sixty seconds, this test thus provides a simple means of determining the suitability of a plate of given composition or thickness for the purpose. The flame of an oxy-acetylene torch is generally accepted to be 6800° F., which, of course, is approximately twice the temperature at which steel usually is poured.

The invention also contemplates smirch plates in which a layer of calcium carbide is embraced within or upon the outer laminations or lamination at one or both sides of the plate, whereby the calcium carbide layer effectively constitutes an interface between the stool and the ingot metal. To provide such a smirch plate, calcium carbide of powdery consistency may be sprinkled between the outermost laminations at one or both sides of the sheet during their assembly and prior to curing so as to become firmly bound between the sheets during curing under heat and pressure. In similar manner, a layer of calcium carbide may be provided as the outermost face at one or both sides of the plate by placing powdered calcium carbide upon the plate prior to curing in the press. The resinous binder which is present at the outermost sheet layer holds the calcium carbide in place after curing, or, if desired, a thin sheet of paper may be laid over the outermost layer to protect the carbide powder against dislodgment prior to use. In place of calcium carbide powder, refractory fillers or parting compositions commonly used in foundry practice may be employed.

Having described my invention, I claim:

1. The method of casting a metal ingot, which method comprises placing a plate having a thickness of from approximately  $\frac{1}{8}$  to  $\frac{1}{4}$  of an inch and made of resin-bonded asbestos fibers arranged in densely compacted relationship on the surface of a stool, superimposing an ingot mold upon the stool in position to embrace the plate over an area which is normally engageable by a stream of molten metal poured into the mold and then pouring molten metal into the mold so that it falls upon the plate, whereby the plate prevents cratering of the stool and adhesion of the ingot metal thereto.

2. The method of casting an ingot, which method comprises placing a plate of densely compacted asbestos fibers bonded together by phenolic resin upon the upper surface of a stool, said plate having a thickness of from approximately  $\frac{1}{8}$  to  $\frac{1}{4}$  of an inch, superimposing an ingot mold upon the stool in a position to embrace the said plate over an area which is normally engageable by a stream of molten metal poured into the mold, then pouring molten metal into the mold so that it falls upon the said plate, whereby the plate protects the stool against cratering and adhesion of the ingot metal thereto.

3. The method of casting a metal ingot, which method comprises placing a plate made of resin-bonded asbestos fibers arranged in densely compacted relationship on the surface of a stool, superimposing an ingot mold upon the stool in position to embrace the plate over an area which is normally engageable by a stream of molten metal poured into the mold and then pouring molten metal into the mold so that it falls upon the plate, whereby the plate prevents cratering of the stool and adhesion of the ingot metal thereto.

## References Cited in the file of this patent

| UNITED STATES PATENTS |                              |
|-----------------------|------------------------------|
| 661,549               | Parks ----- Nov. 13, 1900    |
| 2,128,097             | Mains ----- Aug. 23, 1938 5  |
| 2,249,275             | Hanley ----- July 15, 1941   |
| 2,445,415             | Anderson ----- July 20, 1948 |

## FOREIGN PATENTS

|         |                                  |
|---------|----------------------------------|
| 256,306 | Great Britain ----- Aug. 3, 1926 |
| 810,061 | Germany ----- Aug. 6, 1951       |